

## UNITED STATES PATENT OFFICE

2,396,636

## CASTING OF RARE EARTH METALS

Harold Marland Broadhurst, Liverpool, England,  
assignor to Imperial Chemical Industries Limited,  
a corporation of Great Britain

No Drawing. Application July 7, 1944, Serial No.  
543,950. In Great Britain August 4, 1943

2 Claims. (Cl. 22—200)

This invention relates to improvements in casting rare earth metals and alloys thereof, and to moulds therefor.

Rare earth metal alloys can be cast into flints for pyrophoric lighters by pouring a molten alloy or mixture of iron and mischmetall, with or without additions of small amounts of other metals, into appropriately sized moulds constructed of a ferrous metal shaped to produce sticks of small diameter. The sticks are subsequently broken into small pieces for use. Made in this way the flints have a rough or unpolished surface and may disintegrate on storage, possibly from attack by the atmosphere. It has been proposed to cast rare earth metals from beneath a protecting layer of molten salt into a mould dusted or otherwise coated with magnesia or other inert material such as rolling scale or tin plating so that the pieces of cast metal may be easily removed from the mould.

According to the present invention a process for the production of rare earth metal alloy flints suitable for pyrophoric lighters includes the step of casting the rare earth metal alloy in a ferrous metal mould the surface layers of which mould coming into contact with the molten alloy have been converted by treatment under oxidising conditions to a substantially continuous film of black iron oxide. Advantageously, the treatment under oxidising conditions comprises passing air or steam over the surfaces of the mould maintained at an elevated temperature.

I have found that when flints are cast in a metal mould which has been treated by the method of the present invention it is not only possible to remove the flints from the mould readily, but in addition the stability of the flints in air is considerably increased, and the flints have a more attractive appearance.

In one method of carrying out the invention the moulds are heated in a vessel to a dull red heat and air is blown through the vessel so as to

pass over the surfaces of the mould until the surface layers are oxidised to the black magnetic oxide. The temperature of the air should be controlled so that the mould does not become too hot during the oxidation and cause general break up or loss of shape of the mould. The moulds may then be allowed to cool and can then be used by pouring the molten alloy, for example an alloy of mischmetall and iron, into them from a suitable container, and allowing the cast metal to cool off. It is also possible to cast the metal into the moulds before they have cooled completely, for example while they are still at a temperature of the order of 100° C., and the moulds and the casts may then be allowed to cool together. The sticks of metal as removed from the moulds are found to have a smooth, almost black appearance, and have an improved resistance to disintegration in the air.

20 I claim:

1. A process for the production of rare earth metal alloy flints suitable for use in pyrophoric lighters, and having improved resistance to disintegration in the air which includes the step 25 of casting the rare earth metal alloy in a ferrous metal mould, the surface layers of which mould coming into direct contact with the molten alloy have been converted by treatment under oxidising conditions to a substantially continuous film of black iron oxide.

2. A process for the production of flints suitable for use in pyrophoric lighters, and having improved resistance to disintegration in the air which includes the step of casting an alloy of 35 iron and mischmetall in a ferrous metal mould the surface layers of which coming into direct contact with the molten alloy have been converted by treatment under oxidising conditions to a substantially continuous film of black iron oxide.

HAROLD MARLAND BROADHURST.